

## UNITED STATES PATENT OFFICE

2,117,614

## PRODUCTION OF FAST DYEINGS

Karl Koeberle, Heinrich Scholz, and Julius Eisele,  
Ludwigshafen-on-the-Rhine, Germany, as-  
signors to General Aniline Works, Inc., New  
York, N. Y., a corporation of Delaware

No Drawing. Application June 12, 1937, Serial  
No. 147,923. In Germany July 3, 1936

11 Claims. (Cl. 8—5)

The present invention relates to a process of producing fast dyeings.

We have found that fibrous materials can be dyed very fast shades by applying to the fibres acid-soluble compounds free from sulphonic groups, which are capable of coupling and which have affinity for the fibres, in an acid bath and then allowing solutions of diazo compounds of cyclic amino compounds to act on the fibres thus treated.

Compounds suitable for the process are for example aza compounds of high molecular weight containing hydroxy or amino groups and also amides of cyclic hydroxycarboxylic, or of keto-carboxylic acids containing aza groups, provided the said compounds are soluble in acid and capable of coupling and have affinity for fibres.

The dyeings are produced by first treating the fibrous materials in an acid bath, the acid content of which varies according to the nature of the compound used and may frequently be quite small, with a compound of the aforementioned kind and then treating them with a second bath containing the diazo compound. In this case also it is preferable to select compounds containing no water-solubilizing groups. In many cases it is favorable to carry out the treatment of the fibres in the presence of the usual assistants for the dyeing industry, for example with the co-employment of agents having wetting and/or dispersing action. In this way even compounds of the aforementioned kind which are soluble in acid only with comparative difficulty may be used for the process because any excess of acid such as would be injurious to the fibres can thus be avoided.

The dyeings and prints such as may be obtained according to this invention on various materials, as for example on wool and/or silk, leather, cotton, linen, hemp or artificial fibres, are distinguished in particular by very good fastness to moisture. By suitably selecting the initial materials it is possible to produce a great variety of shades of color. The dyeings have from good to very good fastness to light and weather and are frequently distinguished by a specially good fastness to rubbing.

Dyeings have already been produced on fibrous materials by treating the fibres with compounds capable of coupling and then developing the dyeings by the action of aromatic diazo compounds. The compounds capable of coupling hitherto used, however, have either been insoluble in acid, in which case they have had to be applied to the fibres from alkaline baths, or they have con-

tained sulphonic acid groups, in which case the dyeings obtained had but slight fastness to moisture. Thus according to the known processes it has been impossible to produce fast dyeings on fibrous materials sensitive to alkalies. The process according to this invention, on the other hand, renders it possible to dye in an advantageous manner not only fibres which are sensitive to alkali alone, but in particular also mixed fabrics containing fibres insensitive to alkali and also fibres sensitive to alkali, the resulting dyeings having not only good general fastness but in particular also excellent uniformity. Moreover there is the further advantage that the dyeing may be carried out simultaneously with any desired application of a dyestuff or substance for improving fibres which is only capable of use in an acid bath.

The following examples will further illustrate how the said invention may be carried out in practice but the invention is not restricted to these examples.

## Example 1

50 grams of a mixed fabric of wool and artificial silk are treated for about half an hour at 50° C. in a bath containing per litre 5 grams of 9-methylamino-4-azaphenanthrene and 10 cubic centimetres of 85 per cent formic acid. The fabric thus treated is then brought into a bath containing per litre 2 grams of the diazo compound of 4-chlor-3-aminobenzotrifluoride, the dyeing being developed for about half an hour at 25° C. After hydroextraction, the fabric is rinsed with cold water and the dyeing finished off in the usual way. A clear scarlet-red dyeing of excellent fastness is obtained, the uniformity and fastness to washing and rubbing being especially good.

If 9-dimethylamino - 4 - azaphenanthrene be used instead of 9-methylamino-4-azaphenanthrene, and diazotized 1-amino-4-nitrobenzene be used as the diazo compound, a violet dyeing is obtained.

Fast dyeings may be produced in a corresponding manner on mixed fabrics of cotton and wool or fabrics of unitary fibres.

## Example 2

50 grams of a mixed fabric of cotton and wool or artificial silk or cellulose wool are treated for half an hour at 50° C. in a bath containing per litre 4 grams of 9-acetoacetylarnino-4-azaphenanthrene and 10 cubic centimetres of 10 per cent sulphuric acid. The fabric thus treated is then introduced into a bath containing per litre 2

*Example 5*

grams of diazotized 1-methyl-2-amino-4-chlorbenzene, the dyeing being developed for half an hour at 20° C. After rinsing, the fabric is treated for half an hour at the boiling temperature with 5 a bath containing per litre 2 grams of a non-alkaline washing agent and 0.25 gram of sodium hydrosulphite. A beautiful yellow dyeing is obtained which is distinguished in particular by excellent fastness to washing, rubbing, light and 10 weather. By varying the conditions during the bottoming or developing, it is possible, for example in the case of mixed fabrics, to effect a more or less strong dyeing of the wool as compared with the other fibres. For example the temperature of one of the baths or the amount of acid in 15 the bottoming bath may be increased.

Instead of acetoacetyl-9-amino-4-azaphenanthrene, there may also be used hydroxycarboxylic acid amides of aza compounds. By development 20 with diazo compounds, dyeings are thus obtained having a great variety of shades of color.

*Example 3*

50 grams of a fabric of cotton and/or wool 25 and/or artificial silk are treated for half an hour at 50° C. in a bath containing per litre 4 grams of aminohydroxy-4-azaphenanthrene (obtained by treating 1,3-dihydroxy-4-azaphenanthrene with aqueous ammonia under pressure) and 10 30 cubic centimetres of 85 per cent formic acid. The fabric thus treated is introduced into a bath containing per litre 2 grams of diazotized 1-amino-3-methyl-4-cyano-6-chlorbenzene, the dyeing being developed for half an hour at 30° C. 35 After hydroextraction, the fabric is rinsed with cold water and the dyeing finished off in the usual manner. It is golden-yellow and very fast to washing, rubbing and light.

Dyeings having a great variety of shades are 40 obtained by using, instead of the diazo compounds specified in Examples 1 to 3, other diazo compounds, as for example of 1-amino-2,5-dichlorbenzene, 1-amino-2-methoxy-5-benzyl-sulphone-benzene, 3-amino-4-methoxy-1-ethyl-sulphone-benzene, 1-nitro-2-amino-benzene, 1-methyl-2-amino-5-chlorbenzene, 1-methyl-2-amino-5-nitrobenzene, 1-amino-3-chlorbenzene, 2-amino-diphenyl-sulphone, 1-methyl-3-nitro-4-aminobenzene, 1-trifluormethyl-3-aminophenyl-4-ethyl-sulphone, 1-amino-2-trifluormethyl-4-chlorbenzene, 4-amino-4'-methoxy-diphenylamine, 4-amino-diphenylamine, 1-methoxy-2-amino-5-nitrobenzene, 1-methoxy-3-nitro-4-aminobenzene, 1-amino-4-benzoylaminio-2,5-dimethoxy-benzene, 3-methoxy-4-aminodiphenylamine, 4,4'-diamino-3,3'-dimethoxydiphenyl, 1-amino-4-benzoylaminio-2,5-diethoxybenzene and 55 1-methyl-3-amino-4-methoxy-6-benzoylaminobenzene.

*Example 4*

60 50 grams of a mixed fabric of 75 per cent wool and 25 per cent staple fibre ("Zellwolle") are treated in a bath containing per litre 6 grams of 2',3'-hydroxynaphthoyl-2-amino-pyridine and 150 cubic centimetres of 10 per cent sulphuric acid for half an hour at 50° C. The fabric thus treated is then introduced into a bath containing per litre the diazo compound of 3 grams of 4,4'-dichlor-2-aminodiphenylether. The dyeing 65 is developed at between 40 and 50° C. during 30 minutes, and the fabric is rinsed and treated for half an hour at boiling temperature in a bath containing per litre 2 grams of a non-alkaline washing agent. The fabric is dyed a strong red 70 shade having good fastness properties.

50 grams of a mixed fabric of 75 per cent wool and 25 per cent staple fibre ("Zellwolle") are treated in a bath which contains per litre 6 5 grams of 1-quinolyl-3-methyl-5-pyrazolone (obtainable by reacting 8-hydrazinoquinoline with acetic acid ester) and 24 cubic centimetres of 30 per cent acetic acid, at 50° C. for half an hour. The fabric thus treated is then introduced into a 10 bath containing per litre the diazo compound of 3 grams of 1-methyl-2-amino-4-chlorbenzene, the dyeing being developed for 30 minutes at between 20 and 30° C., and treated in a bath for 30 minutes at the boiling temperature which bath contains per litre 2 grams of a non-alkaline washing agent. The fabric is dyed an intense reddish-yellow shade. The wool and the staple fibre are 15 uniformly covered.

What we claim is:—

1. A process of producing fast dyeings which 20 comprises treating in an acid bath the material to be dyed with aza compounds free from sulphonate groups which have affinity for the said material and are capable of coupling, and then allowing solutions of diazo compounds to act on 25 the fibres thus treated.

2. A process of producing fast dyeings which 30 comprises treating in an acid bath the material to be dyed with aza compounds free from sulphonate groups having at least three rings which have affinity for the said material and are capable of coupling, and then allowing solutions of diazo compounds to act on the fibres thus treated.

3. A process of producing fast dyeings which 35 comprises treating in an acid bath the material to be dyed with aminoazaphenanthrenes free from sulphonate groups which have affinity for the said material and are capable of coupling, and then allowing solutions of diazo compounds to 40 act on the fibres thus treated.

4. A process of producing fast dyeings which 45 comprises treating in an acid bath the material to be dyed with 9-aminoazaphenanthrene and then allowing solutions of diazo compounds to act on the fibres thus treated.

5. A process of producing fast dyeings which 50 comprises treating in an acid bath the material to be dyed with acylaminoazaphenanthrenes free from sulphonate groups which have affinity for the said material and are capable of coupling, and then allowing solutions of diazo compounds to act on the fibres thus treated.

6. A process of producing fast dyeings which 55 comprises treating in an acid bath the material to be dyed with acylaminoazaphenanthrenes the acyl group of which is that of an enolizable keto carboxylic acid, and then allowing solutions of diazo compounds to act on the fibres thus treated.

7. A process of producing fast dyeings which 60 comprises treating in an acid bath the material to be dyed with acetoacetylaminoazaphenanthrenes, and then allowing solutions of diazo compounds to act on the fibres thus treated.

8. A process of producing fast dyeings which 65 comprises treating in an acid bath the material to be dyed with 9-acetoacetylaminoazaphenanthrene, and then allowing solutions of diazo compounds to act on the fibres thus treated.

9. A process of producing fast dyeings which 70 comprises treating in an acid bath the material to be dyed with amides of cyclic hydroxy carboxylic acids capable of coupling having at least one aza group in the molecule, and then allowing 75

solutions of diazo compounds to act on the fibres thus treated.

10. A process of producing fast dyeings which comprises treating in an acid bath the material to be dyed with amides of aromatic ortho-hydroxy carboxylic acids capable of coupling having at least one aza group in the molecule, and then allowing solutions of diazo compounds to act on the fibres thus treated.
10. 11. A process of producing fast dyeings which

comprises treating in an acid bath the material to be dyed with amides of 2-hydroxynaphthalene-3-carboxylic acid containing in the amido group the radical of an aza compound, and then allowing solutions of diazo compounds to act on the fibres thus treated.

KARL KOEBERLE.  
HEINRICH SCHOLZ.  
JULIUS EISELE.

10